

June 7, 1966

R. E. SMITH ET AL

3,254,762

CONDITIONING OF GRANULAR POTASH

Filed Feb. 19, 1962



FIG. 1



FIG. 2

INVENTOR.  
RANDAL E. SMITH  
CLARENCE W. EGBOM  
BY

*M. G. Edwards*  
Attorneys

1

3,254,762

**CONDITIONING OF GRANULAR POTASH**  
Randal E. Smith and Clarence W. Egbom, Carlsbad,  
N. Mex., assignors to Potash Company of America,  
Carlsbad, N. Mex., a corporation of Colorado  
Filed Feb. 19, 1962, Ser. No. 174,108  
17 Claims. (Cl. 209—2)

This invention relates to the reagent conditioning of coarse sylvite ores and particularly to an improved method of conditioning such ores prior to flotation.

In the Carlsbad basin potash ores consisting principally of sylvinitite, which is a mechanical mixture of sylvite and halite with clay and traces of other minerals, are generally upgraded by the flotation process. The flotation process consists of grinding; sizing; scrubbing; desliming; dewatering, which includes removal of brine; conditioning with reagents; and flotation of the sylvite fraction by air bubble attachment.

Initial sizing is generally performed by dry screening into a coarse fraction of about  $-6 +20$  mesh and a standard fraction of minus 20 mesh (Tyler mesh size). The coarse and standard fractions are usually treated separately and this invention is directed primarily to the treatment of the coarse fraction.

The reagent conditioning of coarse sylvite ores is a mixing operation in which amine and oil reagents are added to a pulp following scrubbing and slime removal operations. The amine reagent is well known in the art of potash flotation. The preferred reagent for coarse flotation is in general based on octadecyl amine, but consists of mixtures prepared from natural fats with or without further hydrogenation. A common reagent is known as tallow amine, and the common reagent for coarse flotation is a hydrogenated tallow amine. This reagent is preferably added as an emulsion prepared by partial neutralization with acid.

The oils may be crude residues from petroleum refining and are generally heavy or viscous in character. Such viscous reagents are difficult to distribute thoroughly in the slurry. It is recognized in the industry that gentle mixing for as short a time as possible is desirable in coarse sylvite conditioning, since increasing the time or intensity of the mixing or both may result in further slimes release or the production of fine particles by attrition, both of which consume additional reagent and have other undesirable effects. However, in many instances, gentle mixing in conventional fashion does not provide the thorough reagent distribution necessary for effective flotation of coarse potash.

It has now been found that reagents can be added in the presence of considerable brine, provided the excess brine is removed before the pulp is fed to the flotation cell. We have found that the best results are attained when the reagents are added to a pulp containing about 15% or more brine by weight. Gentle mixing following brine removal has also been found to be effective in improving flotation efficiency.

Substantial improvements in flotation efficiency which may be observed as lower reagent rates or larger particles floated or both, are made possible by use of this method. It is particularly advantageous at low rates of reagent use.

It is an object of our invention to provide a simple, economical and efficient preparation or conditioning of potash ores for flotation treatment which provides a low rate of reagent use in highly efficient flotation concentration.

Another object of this invention is to provide a simple,

2

economical and efficient preparation or conditioning of coarse potash ores for flotation treatment which provides a highly efficient flotation concentration of larger particles.

5 A further object of our invention is to provide a rapid and efficient filming or coating of coarse potash ore particles without appreciable size reduction of particles by attrition.

Still another object of this invention is to provide a simple, economical and efficient preparation or conditioning of coarse potash ores which provides a highly efficient flotation concentration without use of a clay blinding reagent in the treatment.

The practice of our invention will be described with reference to the accompanying drawings. In the drawings:

FIG. 1 is a typical flow sheet for the practice of our invention utilizing a single reagent mixing stage; and

FIG. 2 is a typical flow sheet for the practice of our invention utilizing a two-stage mixing of reagent.

20 The flow sheet of FIG. 1 depicts a typical practice where only a single stage mixing treatment is required. As shown, cleaned and deslimed ore from a suitable source of supply 3 is delivered into a mechanical mixer 4, preferably a horizontal rotary drum providing a retention time of from about 20 seconds to about 1 minute. An amine collector reagent 5 and an oil 6, if desired, are fed into mixer 4 in controlled quantities. A major portion of the brine is removed from the ore, usually by gravity draining as on screen 7, and the separated brine 30 may be returned to brine clarification.

The conditioned ore after brine removal is delivered as the feed 8 to a flotation stage 9 in which brine of the ore 10 is provided as the carrier vehicle in the flotation action. Coarse potash collects on the surface of the brine 35 and is removed as a concentrate at 11, while the flotation tailings are removed as indicated at 12. Both concentrate and tailings may be further processed as known in the art.

The circuit shown in FIG. 2 is essentially the same as the one just described, except for the two-stage mixing. 40 After initially mixing at stage 4 and dewatering as indicated at 7, the ore is fed into a second mixer 4<sup>1</sup> also providing gentle mixing for an interval of about a minute or less, and the second mixer discharge is fed to the flotation stage 9.

45 It is understood when referring to brine, we mean a solution prepared by contact with the ore, and which is approximately saturated with NaCl and KCl and which is used as the fluid medium in the sylvite ore dressing process.

50 Dewatering as used herein designates a liquid-solids separation in which associated brine is separated from the ore.

In practicing the invention the coarse sylvite ore is prepared by crushing and screening the ore to obtain a 55 particle size range that is substantially  $-6 +20$  mesh. The ore is slurried in brine and scrubbed to release clay slimes. The pulp is then deslimed by washing with clean brine to remove all free slimes, leaving a clean pulp which is ready for reagent conditioning.

60 In our method, the clean pulp is delivered to the conditioner at a pulp density from 50% to 85% solids, preferably about 65% solids. The conditioning vessel is preferably a revolving horizontal drum, turning at a rate to give gentle but thorough mixing. The amine reagent and the oil are added and the pulp is mixed for  $\frac{1}{2}$  to 1 minute, with the shorter time usually sufficient for complete reagent distribution. If the conditioner revolves too rapidly or if the retention time is too long, further slimes 65 may be released causing a greater demand for reagents.

The presence of brine in this part of the conditioning process is of value as a lubricant to further gentle the mixing action and to distribute small quantities of reagents through the pulp.

The pulp is then partially dewatered. This can be ac-

formed on the carefully mixed lot of sylvinite ore from the Carlsbad, New Mexico basin. No auxiliary reagents such as starch or guar were used.

Table I contains typical examples of the effect of removing brine after initial mixing without further mixing.

TABLE I

| Percent 1st<br>Pulp<br>Density | Mix<br>Time,<br>Sec. | Drain    | Final<br>Pulp<br>Density | Reagent Rates,<br>Lb./Ton |     | Temp.,<br>°F. | Tailing<br>Grade, Per-<br>cent K <sub>2</sub> O | Percent<br>KCl<br>Recovery |
|--------------------------------|----------------------|----------|--------------------------|---------------------------|-----|---------------|-------------------------------------------------|----------------------------|
|                                |                      |          |                          | Amine                     | Oil |               |                                                 |                            |
| 65                             | 60                   | No-----  | 65                       | 0.1                       | 0.6 | 77            | 11.01                                           | 64.0                       |
| 65                             | 60                   | Yes----- | 93                       | 0.1                       | 0.6 | 77            | 4.28                                            | 87.6                       |
| 75                             | 60                   | No-----  | 75                       | 0.06                      | 0.8 | 85            | 6.77                                            | 76.3                       |
| 75                             | 60                   | Yes----- | 95                       | 0.06                      | 0.8 | 85            | 3.03                                            | 89.9                       |
| 50                             | 60                   | No-----  | 50                       | 0.06                      | 0.8 | 85            | 9.00                                            | 66.7                       |
| 50                             | 60                   | Yes----- | 75                       | 0.06                      | 0.8 | 85            | 7.10                                            | 74.4                       |

complished by draining by gravity through a screen or by 20 suction or other mechanical means. The pulp is drained to 85% solids or above with the preferred density being

Table II illustrates the effect of draining to different pulp densities after initial mixing at uniform low pulp densities.

TABLE II

| Percent 1st<br>Pulp<br>Density | Mix<br>Time,<br>Sec. | Drain    | Final<br>Pulp<br>Density | Reagent Rates,<br>Lb./Ton |     | Temp.,<br>°F. | Tailing<br>Grade, Per-<br>cent K <sub>2</sub> O | Percent<br>KCl<br>Recovery |
|--------------------------------|----------------------|----------|--------------------------|---------------------------|-----|---------------|-------------------------------------------------|----------------------------|
|                                |                      |          |                          | Amine                     | Oil |               |                                                 |                            |
| 50                             | 60                   | No-----  | 50                       | 0.06                      | 0.8 | 85            | 9.00                                            | 66.7                       |
| 50                             | 60                   | Yes----- | 75                       | 0.06                      | 0.8 | 85            | 7.10                                            | 74.4                       |
| 50                             | 60                   | Yes----- | 85                       | 0.06                      | 0.8 | 85            | 4.20                                            | 86.3                       |
| 50                             | 60                   | Yes----- | 95                       | 0.06                      | 0.8 | 85            | 4.05                                            | 86.7                       |

above 90%. This may take from 20 seconds to over 1 35 minute by gravity depending on the depth of the ore bed, reagent rates, particle size, etc.

Table III illustrates the advantage gained in a typical test in which a period of mixing was given the ore following draining of the brine used in the mixing step.

TABLE III

| Percent 1st<br>Pulp Density | 1st Mix<br>Time, Sec. | Drain    | 2nd Mix<br>Time, Sec. | Final Pulp<br>Density | Reagent Rates,<br>Lb./Ton |     | Temp.,<br>°F. | Tailing<br>Grade, Per-<br>cent K <sub>2</sub> O | Percent KCl<br>Recovery |
|-----------------------------|-----------------------|----------|-----------------------|-----------------------|---------------------------|-----|---------------|-------------------------------------------------|-------------------------|
|                             |                       |          |                       |                       | Amine                     | Oil |               |                                                 |                         |
| 65                          | 60                    | Yes----- | -----                 | 93                    | 0.1                       | 0.6 | 77            | 4.28                                            | 87.6                    |
| 65                          | 30                    | Yes----- | 30                    | 93                    | 0.1                       | 0.6 | 77            | 2.88                                            | 91.9                    |

As the brine is drained from the pulp the solids may be mixed gently. Flotation of the prepared ore provides improved recovery over that at identical reagent rates without draining, or, comparable flotation is achieved at

50 Table IV contains a number of general examples showing the advantage of draining after initial mixing over not draining at various levels of reagent use, different starting pulp densities and at two different temperatures.

TABLE IV

| Percent 1st<br>Pulp Density | 1st Mix<br>Time, Sec. | Drain    | 2nd Mix<br>Time, Sec. | Final Pulp<br>Density | Reagent Rates,<br>Lb./Ton |     | Temp.,<br>°F. | Tailing<br>Grade, Per-<br>cent K <sub>2</sub> O | Percent KCl<br>Recovery |
|-----------------------------|-----------------------|----------|-----------------------|-----------------------|---------------------------|-----|---------------|-------------------------------------------------|-------------------------|
|                             |                       |          |                       |                       | Amine                     | Oil |               |                                                 |                         |
| 65                          | 30                    | No-----  | 30                    | 65                    | 0.075                     | 0.6 | 77            | 7.39                                            | 77.3                    |
| 65                          | 30                    | Yes----- | 30                    | 93                    | 0.075                     | 0.6 | 77            | 3.50                                            | 90.0                    |
| 65                          | 30                    | No-----  | 30                    | 65                    | 0.15                      | 1.0 | 77            | 7.10                                            | 78.7                    |
| 65                          | 30                    | Yes----- | 30                    | 93                    | 0.15                      | 1.0 | 77            | 2.61                                            | 92.6                    |
| 75                          | 30                    | No-----  | 30                    | 75                    | 0.15                      | 1.0 | 77            | 4.58                                            | 86.4                    |
| 75                          | 30                    | Yes----- | 30                    | 93                    | 0.15                      | 1.0 | 77            | 2.84                                            | 91.9                    |
| 75                          | 30                    | No-----  | 30                    | 75                    | 0.15                      | 0.6 | 90            | 8.27                                            | 70.7                    |
| 75                          | 30                    | Yes----- | 30                    | 93                    | 0.15                      | 0.6 | 90            | 3.01                                            | 90.5                    |
| 75                          | 30                    | No-----  | 30                    | 75                    | 0.2                       | 0.8 | 90            | 4.29                                            | 85.6                    |
| 75                          | 30                    | Yes----- | 30                    | 93                    | 0.2                       | 0.8 | 90            | 2.58                                            | 91.2                    |
| 65                          | 30                    | No-----  | 30                    | 65                    | 0.2                       | 0.8 | 90            | 5.53                                            | 82.0                    |
| 65                          | 30                    | Yes----- | 30                    | 93                    | 0.2                       | 0.8 | 90            | 1.93                                            | 93.9                    |

substantially reduced reagent rates when the reagentized ore is dewatered.

To illustrate the advantages of the invention, the following flotation results are tabulated. All tests were per-

50 Table V illustrates the combined effect of initial mixing at low pulp density, followed by draining and further mixing over conventional conditioning. Results are shown at two different reagent rates.

TABLE V

| Percent 1st<br>Pulp Density | 1st Mix<br>Time, Sec. | Drain    | 2nd Mix<br>Time, Sec. | Final Pulp<br>Density | Reagent Rates,<br>Lb./Ton |     | Temp.,<br>° F. | Tailings<br>Grade, Per-<br>cent K <sub>2</sub> O | Percent KCl<br>Recovery |
|-----------------------------|-----------------------|----------|-----------------------|-----------------------|---------------------------|-----|----------------|--------------------------------------------------|-------------------------|
|                             |                       |          |                       |                       | Amine                     | Oil |                |                                                  |                         |
| 95                          | 60                    | No-----  |                       | 95                    | 0.1                       | 0.8 | 90             | 7.18                                             | 76.0                    |
| 74                          | 30                    | Yes----- | 30                    | 93                    | 0.1                       | 0.8 | 90             | 4.22                                             | 86.2                    |
| 95                          | 60                    | No-----  |                       | 95                    | 0.2                       | 0.8 | 90             | 2.91                                             | 90.7                    |
| 74                          | 30                    | Yes----- | 30                    | 93                    | 0.2                       | 0.8 | 90             | 2.64                                             | 91.5                    |

We have thus found a distinct improvement in conditioning of these ores by distributing the reagent in a wet pulp, followed by draining off the excess brine.

Since these factors will vary with reagent rates, with temperature, with type of reagent, the times suggested are for explanation only, and we do not intend to be limited by them. Changes and modifications may be availed of within the spirit and scope of the invention as defined in the hereunto appended claims.

What we claim is:

1. A method of preparing potash ores for a flotation treatment, consisting of the steps of forming a pulp of cleaned and deslimed potash ore in a size range of about minus 6 plus 20 mesh and a brine carrier and having a pulp density of about 50% to 85% solids, introducing an amine collector reagent into said pulp, mixing the pulp and reagent so introduced, then moving the pulp and reagent mixture directly into a brine removal stage in which a portion of the brine is removed to establish a pulp density of at least 85% solids and wherein reagentized ore surfaces are exposed to atmosphere, and passing the reagentized ore after brine removal without further treatment into a flotation concentration stage.

2. A method of preparing potash ores for a flotation treatment, consisting of the steps of forming a pulp of cleaned and deslimed potash ore in a size range of about minus 6 plus 20 mesh and a brine carrier and having a pulp density of about 50% to 85% solids, introducing an amine collector reagent into said pulp, mixing the pulp and reagent so introduced without material attrition, then removing the pulp and reagent mixture directly into a brine removal stage in which a portion of the brine is removed to establish a pulp density of at least 85% solids and wherein reagentized ore surfaces are exposed to atmosphere, and passing the reagentized ore after brine removal without further treatment into a flotation concentration stage.

3. A method of preparing potash ores for a flotation treatment, consisting of the steps of forming a pulp of cleaned and deslimed potash ore in a size range of about minus 6 plus 20 mesh and a brine carrier and having a pulp density of about 50% to 85% solids, introducing an amine collector reagent into said pulp, mixing the pulp and reagent so introduced for from about 20 seconds to about one minute, then moving the pulp and reagent mixture directly into a brine removal stage in which a portion of the brine is removed to establish a pulp density of at least 85% solids and wherein reagentized ore surfaces are exposed to atmosphere, and passing the reagentized ore after brine removal without further treatment into a flotation concentration stage.

4. A method of preparing potash ores for a flotation treatment, consisting of the steps of forming a pulp of cleaned and deslimed potash ore in a size range of about minus 6 plus 20 mesh and a brine carrier and having a pulp density of about 50% to 85% solids, introducing an amine collector reagent into said pulp, mixing the pulp and reagent so introduced, then moving the pulp and reagent mixture directly into a brine removal stage in which a portion of the brine is removed to establish a pulp density of more than 85% solids and wherein reagentized ore surfaces are exposed to atmosphere, and passing the reagentized ore after brine removal without further treatment into a flotation concentration stage.

5. A method of preparing potash ores for a flotation treatment, consisting of the steps of forming a pulp of cleaned and deslimed potash ore in a size range of about minus 6 plus 20 mesh and a brine carrier and having a pulp density of about 50% to 85% solids, introducing an amine collector reagent into said pulp, mixing the pulp and reagent so introduced for about one minute, then moving the pulp and reagent mixture directly into a brine removal stage in which a portion of the brine is removed to establish a pulp density of at least 85% solids and wherein reagentized ore surfaces are exposed to atmosphere, and passing the reagentized ore after brine removal without further treatment into a flotation concentration stage.

6. A method of preparing potash ores for a flotation treatment, consisting of the steps of forming a pulp of cleaned and deslimed potash ore in a size range of about minus 6 plus 20 mesh and a brine carrier and having a pulp density of about 50% to 85% solids, introducing an amine collector reagent into said pulp, mixing the pulp and reagent so introduced, then moving the pulp and reagent mixture directly into a brine drainage stage in which a portion of the brine is removed to establish a pulp density of at least 85% solids and wherein reagentized ore surfaces are exposed to atmosphere, and passing the reagentized ore after brine removal without further treatment into a flotation concentration stage.

7. A method of preparing potash ores for a flotation treatment, consisting of the steps of forming a pulp of cleaned and deslimed potash ore in a size range of about minus 6 plus 20 mesh and a brine carrier and having a pulp density of about 50% to 85% solids, introducing an amine collector reagent into said pulp, mixing the pulp and reagent so introduced, then moving the pulp and reagent mixture directly into a brine removal stage in which a portion of the brine is removed to establish a pulp density of about 90% solids and wherein reagentized ore surfaces are exposed to atmosphere, and passing the reagentized ore after brine removal without further treatment into a flotation concentration stage.

8. A method of preparing potash ores for a flotation treatment, consisting of the steps of forming a pulp of cleaned and deslimed potash ore in a size range of about minus 6 plus 20 mesh and a brine carrier and having a pulp density of about 50% to 85% solids, introducing an amine collector reagent into said pulp, mixing the pulp and reagent so introduced without blinding reagent addition, then moving the pulp and reagent mixture directly into a brine removal stage in which a portion of the brine is removed to establish a pulp density of at least 85% solids and wherein reagentized ore surfaces are exposed to atmosphere, and passing the reagentized ore after brine removal without repulping into a flotation concentration stage.

9. A method of preparing potash ores for a flotation treatment, consisting of the steps of forming a pulp of cleaned and deslimed potash ore in a size range of about minus 6 plus 20 mesh and a brine carrier and having a pulp density of about 50% to 85% solids, introducing an amine collector reagent into said pulp, mixing the pulp and reagent so introduced, then moving the pulp and reagent mixture directly into a brine removal stage in which a portion of the brine is removed to establish a pulp density of at least 85% solids and wherein reagentized ore surfaces are exposed to atmosphere, and

passing the reagentized ore after brine removal and at said established density into a flotation concentration sage.

10. A method of preparing potash ores for a flotation treatment, consisting of the steps of forming a pulp of cleaned and deslimed potash ore in a size range of about minus 6 plus 20 mesh and a brine carrier and having a pulp density of about 50% to 85% solids, introducing an amine collector reagent into said pulp, mixing the pulp and reagent so introduced, then moving the pulp and reagent mixture directly into a brine removal stage in which a portion of the brine is removed to establish a pulp density of at least 85% solids and wherein reagentized ore surfaces are exposed to atmosphere, and passing the reagentized ore after final mixing without further treatment into a flotation concentration stage.

11. A method of preparing potash ores for a flotation treatment, consisting of the steps of forming a pulp of cleaned and deslimed potash ore in a size range of about minus 6 plus 20 mesh and a brine carrier and having a pulp density of about 50% to 85% solids, introducing an amine collector reagent into said pulp, mixing the pulp and reagent so introduced without blinding reagent addition, then moving the pulp and reagent mixture directly into a brine removal stage in which a portion of the brine is removed to establish a pulp density of at least 85% solids and wherein reagentized ore surfaces are exposed to atmosphere, subjecting the ore and said reagent to additional mixing after brine removal, and passing the reagentized ore after final mixing directly into a flotation concentration stage.

12. A method of preparing potash ores for a flotation treatment, consisting of the steps of forming a pulp of cleaned and deslimed potash ore in a size range of about minus 6 plus 20 mesh and a brine carrier and having a pulp density of about 50% to 85% solids, introducing an amine collector reagent into said pulp, mixing the pulp and reagent so introduced for from about 20 seconds to about one minute, then moving the pulp and reagent mixture directly into a brine removal stage in which a portion of the brine is removed to establish a pulp density of at least 85% solids and wherein reagentized ore surfaces are exposed to atmosphere, mixing the ore at said density with said reagent for from 20 seconds to about one minute, and passing the reagentized ore after final mixing without further treatment into a flotation concentration stage.

13. A method of preparing potash ores for a flotation treatment, consisting of the steps of forming a pulp of cleaned and deslimed potash ore in a size range of about minus 6 plus 20 mesh and a brine carrier and having a pulp density of about 50% to 85% solids, introducing an amine collector reagent into said pulp, mixing the pulp and reagent mixture directly into a brine removal stage in which a portion of the brine is removed to establish a pulp density of at least 90% solids and wherein reagentized ore surfaces are exposed to atmosphere, subjecting the ore and said reagent to additional mixing after brine removal, and passing the reagentized ore after final mixing without further treatment into a flotation concentration stage.

14. A method of preparing potash ores for a flotation treatment, consisting of the steps of forming a pulp of

cleaned and deslimed potash ore in a size range of about minus 6 plus 20 mesh and a brine carrier and having a pulp density of about 65% solids, introducing an amine collector reagent into said pulp, mixing the pulp and reagent so introduced, then moving the pulp and reagent mixture directly into a brine removal stage in which a portion of the brine is removed to establish a pulp density of at least 85% solids and wherein reagentized ore surfaces are exposed to atmosphere, and passing the reagentized ore after brine removal without further treatment into a flotation concentration stage.

15. A method of preparing potash ores for a flotation treatment, consisting of the steps of forming a pulp of cleaned and deslimed potash ore in a size range of about minus 6 plus 20 mesh and a brine carrier and having a pulp density of about 65% solids, introducing an amine collector reagent into said pulp, mixing the pulp and reagent so introduced, then moving the pulp and reagent mixture directly into a brine drainage stage in which a portion of the brine is removed to establish a pulp density of at least 90% solids and wherein reagentized ore surfaces are exposed to atmosphere, and passing the reagentized ore after brine drainage without further treatment into a flotation concentration stage.

16. A method of preparing potash ores for a flotation treatment, consisting of the steps of forming a pulp of cleaned and deslimed potash ore in a size range of about minus 6 plus 20 mesh and a brine carrier and having a pulp density of about 50% to 85% solids, introducing an amine collector reagent into said pulp, mixing the pulp and reagent so introduced at a first mixing stage, then moving the pulp and reagent mixture directly into a brine removal stage in which sufficient free brine is removed to establish a pulp density of at least 85% solids and wherein reagentized ore surfaces are exposed to atmosphere, moving the reagentized ore after brine removal through a second mixing stage, and passing the reagentized ore after final mixing and at said established density into a flotation concentration stage.

17. A method of preparing potash ores for a flotation treatment, consisting of the steps of forming a pulp of cleaned and deslimed potash ore in a size range of about minus 6 plus 20 mesh and a brine carrier and having a pulp density of about 50% to 85% solids, introducing an amine collector reagent into said pulp, mixing the pulp and reagent so introduced at a first mixing stage, then moving the pulp and reagent mixture directly into a brine removal stage in which sufficient free brine is removed to establish a pulp density of at least 85% solids and wherein reagentized ore surfaces are exposed to atmosphere, moving the reagentized ore after brine removal through a second mixing stage for mixing with said reagent for from about 20 seconds to one minute, and passing the reagentized ore after final mixing and at said established density into a flotation concentration stage.

#### References Cited by the Examiner

#### UNITED STATES PATENTS

2,950,007 8/1960 Smith ----- 209—116

60 FRANK W. LUTTER, *Primary Examiner.*

ROBERT A. O'LEARY, *Examiner.*